

## UNITED STATES PATENT OFFICE

2,380,921

## ZINC BASE ALLOY

Edward S. Bunn, Rome, N. Y., assignor to Revere  
Copper and Brass Incorporated, Rome, N. Y.,  
a corporation of Maryland

No Drawing. Application June 16, 1943.  
Serial No. 491,059

4 Claims. (Cl. 75—178)

My invention, which relates to zinc base alloys and has among its objects the production of a zinc base alloy of improved characteristics, will be best understood from the following description, the scope of the invention being more particularly pointed out in the appended claims.

As will be well understood by those skilled in the art, pure zinc in forms commercially available has a rather low tensile strength, but good ductility. Although capable of being hot and cold worked this metal has the defect that it self anneals when cold worked and thus, as distinguished from most cold workable metals, cannot be hardened and its tensile strength increased by cold working. Further, pure zinc is subject to grain growth as it ages, particularly in hot and humid situations, causing it gradually to lose with age most of its ductility coupled with a serious reduction in its tensile strength. For example, hot rolled zinc having a tensile strength of 17,000 pounds per square inch and a ductility represented by an elongation of 45% in 2 inches will, when subjected to the standard test for determining the effect of age on zinc and its alloys, namely, subjecting it to moist steam at 95° C. for 10 days, have its tensile strength reduced to 11,000 pounds per square inch and its elongation in 2 inches reduced to about 2%, the latter indicating almost total loss of ductility.

To attempt to cure these defects of zinc by adding other elements to it commonly results in either so great a sacrifice of its ductility as to render it unsuitable for most uses or, if its tensile strength and ductility are originally satisfactory when such elements are added to it, its being subject to a serious loss of one or the other, or both, as the zinc ages, and further commonly makes the zinc subject to intergranular corrosion and unstable in respect to dimensions as it ages.

However, applicant has found that grain growth in zinc to an unsatisfactory degree in respect to use of the zinc in most situations can be substantially prevented by adding to it small amounts of copper and substance of the group consisting of tellurium and selenium without causing, to any unsatisfactory degree, for such uses, the other defects mentioned as commonly incident to the attempt to cure grain growth by adding other elements to zinc. At the same time the particular additions mentioned are found to impart to the zinc other properties of great value in commercial application of the resulting alloy.

Applicant has found that by adding copper and tellurium or selenium, or both the latter, to

zinc even in relatively small amounts markedly increases the tensile strength of the zinc without unsatisfactorily decreasing its ductility for most uses of the resulting alloy. This increase in tensile strength is greater than if copper alone is added. For example, adding 1% copper to zinc will increase its tensile strength in the hot rolled condition from 17,000 to 29,000 pounds per square inch, its ductility represented by an elongation of 45% in 2 inches remaining substantially unchanged, but adding 0.2% tellurium or selenium, or a mixture of the two, with 1% copper will further increase the tensile strength of the zinc in the hot rolled condition to 34,000 pounds per square inch, while decreasing its elongation in 2 inches only to about 35%, which latter is a very satisfactory ductility for most uses of the resulting alloy.

Satisfactory results in the above respects will be secured within the ranges of 0.1 to 5% copper and 0.2 to 0.8% metal of the group consisting of tellurium and selenium. Further, the resulting alloys are commercially hot and cold workable by usual mill processes, and by them can be hot or cold rolled into sheets, these alloys being much more readily worked, particularly when cold, than binary zinc-copper alloys, which latter cannot be commercially cold rolled when the amount of copper exceeds about 3 or 4%. The improved worked alloys have a resistance to shock or impact loading very much superior to that of zinc or binary zinc-copper alloys, making them satisfactory for uses where such property is of significance, as it usually is. The tensile strength of the improved alloys likewise is much higher than that of pure zinc and markedly higher than that of binary zinc-copper alloys. Still further, the ductility of the improved alloys is satisfactorily high for most uses, as is also their stability in respect to maintaining good tensile strength and ductility as they age. For any ordinary use of the improved alloys they are satisfactorily stable with age in respect to maintaining their dimensions and freedom from warping, and have good resistance to intergranular corrosion. With amounts of 1.5% or more copper they do not self anneal when cold worked. Best results in respect to securing high tensile strength combined with good ductility are secured within the range of 2.25 to 5% copper. In respect to securing good all around properties of the alloys best results will be had when the amount of metal of the group is not substantially more than 50% of the amount of copper.

It will be understood that, within the scope

of the appended claims, other elements may be added to the improved alloy for modifying its properties or imparting additional properties, so long as the characteristics imparted by adding copper and metal of the group to the zinc are not destroyed. 5

I claim:

1. Zinc base alloys containing, approximately, 0.1 to 5% copper, 0.02 to 0.8% substance of the group consisting of tellurium and selenium, the 10 balance being substantially zinc.

2. Zinc base alloys according to claim 1 having 1.5% or more copper.

3. Zinc base alloys according to claim 1 having 2.25% or more copper.

4. Zinc base alloys according to claim 1 in which the percentage amount of substance of the group of substances is not substantially more than one-half the percentage amount of copper.

EDWARD S. BUNN.